

## UNITED STATES PATENT OFFICE

2,157,146

## SCALE-RESISTING STEEL ALLOY

Gerhard Riedrich, Krefeld-Forstwald, Germany,  
assignor to Deutsche Edelstahlwerke Aktien-  
gesellschaft, Krefeld, Germany, a corporation  
of Germany

No Drawing. Application November 7, 1936, Se-  
rial No. 109,673. In Germany May 19, 1936

## 1 Claim. (Cl. 75—123)

My invention refers to a steel alloy of which, in particular, articles are made which must be highly resistant to scaling.

A steel alloy has already been suggested in the prior art which is composed of 0.01 to 1.50% carbon, 8.00 to 18% chromium, 15.00 to 25% manganese, and more than 3% to 8% silicon, the remainder of the alloy consisting of iron and the usual traces of sulphur, phosphorus and other impurities found in steel alloys. Prior alloys of this character, aside from being scale-resisting, have the advantage that they can be easily worked and machined and do not become brittle when used at high temperatures.

15 The present invention is based on the recognition that the cost of producing such alloys, without impairing the above-mentioned essential characteristics, can be materially reduced by either entirely omitting the content of the costly 20 chromium, or at least reducing its content considerably below that suggested in the prior art. With the reduction of the chromium content the carbon content should also be reduced and be limited to a range of from 0.01 to 0.30%.

25 According to my invention, I propose a scale-  
resisting steel alloy of the following composition:

|           | Per cent        |
|-----------|-----------------|
| Carbon    | 0.01-0.30       |
| Manganese | 15.00-30.00     |
| Silicon   | over 3.00-10.00 |

the remainder of the alloy being composed of iron and the unavoidable traces of impurities such as 35 sulphur and phosphorus. If desired, up to 6%

chromium may be added. Furthermore, if certain additional characteristics of the alloy are desired, small amounts of molybdenum, or tungsten, or titanium, or vanadium, or tantalum, may be added, either alone or a combination of these elements, but in general such additions should not exceed 2% of the alloy. For instance, if it is desired to improve the strength at high temperatures of the article made of my novel alloy, molybdenum or tungsten or both should be added within the above mentioned percentage. If brittleness is to be resisted, titanium, vanadium or tantalum may be added.

The class of articles or tools which are particularly improved when made of my novel alloy are 15 specifically those used in annealing, hardening, and similar high temperature processes, such as annealing boxes or pots, cementing boxes or pots, case-hardening boxes or pots, raking hooks or bars. Further, heat-treating furnace construction elements such as lifting beams, rails for automatic furnaces, grate bars for enameling ovens and similar objects, in all of which cases the equipment when exposed to high temperatures should not only retain its mechanical 20 strength but should resist scaling.

## I claim:

A steel to be exposed to high temperatures in performing metallurgical or other thermal operations, consisting of 0.01% to 0.30% carbon, 25 15.0% to 30.0% manganese, over 3.0% to 10.0% silicon, the remainder iron and customary traces of impurities, and characterized by elevated scale-resistancy.

GERHARD RIEDRICH. 35